

Jan. 12, 1954

F. T. CREGO ET AL  
DESULFURIZATION AND DECARBURIZATION  
OF IRON AND IRON ALLOYS  
Filed May 5, 1949

2,665,982



INVENTORS

FRANCIS T. CREGO

HAROLD R. FISHER

By *Francis T. Crego* *Harold R. Fisher*  
ATTORNEYS

## UNITED STATES PATENT OFFICE

2,665,982

## DESULFURIZATION AND DECARBURIZATION OF IRON AND IRON ALLOYS

Francis T. Crego, East Orange, and Harold R. Fisher, Metuchen, N. J., assignors to Air Reduction Company, Incorporated, New York, N. Y., a corporation of New York

Application May 5, 1949, Serial No. 91,574

2 Claims. (Cl. 75—51)

1

This invention relates to desulphurization of molten iron and iron alloys such as steel, and particularly to the elimination of sulphur in the open hearth process for the production of steel. The invention also relates to the decarburization of molten iron and iron alloys in the open hearth process after the desulphurization thereof. The invention may be applied to the treatment of any molten bath of iron or iron alloys.

Sulphur is a deleterious element which is normally present in iron and steel manufactured by conventional methods, and at least a portion of the sulphur must be removed to produce metal meeting standard specifications and suitable for commercial applications.

The present practice for reducing the sulphur content of iron in the manufacture of steel involves simultaneous removal of carbon. A large excess of lime is added to the slag which, by contact with the metal, causes the sulphur to combine with the lime until an equilibrium condition is established. Decarburization is effected by the addition of iron ore which oxidizes the carbon in the metal. Oxidation does not, however, promote desulphurization of metals. Rather it tends to produce a reversal of the reaction of sulphur and calcium. Reduction of the sulphur content of the metal is, therefore, relatively slow and especially so when the sulphur content is high. It may require from one to three hours to effect sufficient desulphurization of a seventy-ton heat.

It is the object of the present invention to afford a rapid, effective and economical method of eliminating sulphur, or both sulphur and carbon, from molten iron and steel, thereby permitting the attainment of the desired composition in respect to sulphur or sulphur and carbon content in the minimum time.

Other objects and advantages of the invention will be apparent as it is better understood by reference to the following specification and the accompanying drawing, in which the figure represents a cross-section of an open hearth furnace illustrating the application of the invention to the operation of such a furnace.

The invention depends upon the correlation of certain factors including basicity and fluidity of the slag and the agitation of the bath by means of a gas introduced.

We have discovered that the lime to silica ratio, during the desulphurization, must be at least 2.5:1 and the slag must have a high fluidity which is obtained by adding fluorspar in sufficient quantity. Thus, from 500 to 600 pounds

10

15

20

25

30

35

40

45

50

55

2

of fluorspar must be added to the slag employed in a 70-ton basic open hearth steel furnace to properly effect the result. Oxidizing agents are eliminated during the desulphurization operation, since oxidation causes a reversal of the reaction between calcium and sulphur and the return of sulphur to the metal and retards the desulphurizing effect of the calcium present in the slag. Thus no iron ore or other oxidizing agent is employed during the desulphurizing procedure.

To effect the necessary agitation during the desulphurization, we introduce an inert gas such as nitrogen through a suitable pipe, for example an ordinary iron pipe which is inserted through the door of the furnace and through the slag layer into the molten metal. Any inert gas free from oxidizing constituents may be used, such as argon and helium, though these gases are probably too expensive for such use in view of the availability of nitrogen.

A reducing gas can be substituted for nitrogen, or a mixture of inert and reducing gases, for example a mixture of inert and reducing gases, for example a mixture of nitrogen and propane is suitable. The exact proportions of the mixture are not critical, since the principal function of the gas is agitation of the molten metal.

By operating in the manner described, the sulphur content of the metal may be reduced effectively within from ten to twenty minutes, as compared with an hour to three hours by procedures heretofore known. The time is based upon a 70-ton heat in an open hearth furnace and may vary depending upon the type of apparatus used and the quantity of metal involved.

After the desulphurization has proceeded to the desired point, the slag is removed and a new slag is substituted. Decarburization may then be accomplished either by the conventional method of adding iron ore or by the introduction of oxygen through a suitable pipe as in the most modern and effective decarburizing methods.

In the accompanying drawing, we have illustrated an open hearth furnace, although it is to be understood that the invention is not limited to such a furnace, since it may be carried out in any suitable type of metallurgical furnace in which heat may be supplied by combustion, electric arc or otherwise in order to maintain the temperature of the metal.

Referring to the drawing, 5 indicates an open hearth furnace having a roof 6, a hearth 7 and

walls 8, one of the walls having a charging opening 9. It will be understood that the hearth is fired by the combustion of fuel in the conventional manner, although, as indicated, other heating means may be employed. The bath of molten metal 10 on the hearth is covered by a layer of slag 11 which, in accordance with the present invention, includes lime and silica in the proper ratio with the addition of sufficient fluorspar to afford the necessary fluidity. A 10 pipe 12 is inserted through the opening 9 through the slag layer 11 and into the bath of molten metal 10, and a suitable gas, such as nitrogen, other inert gas, a reducing gas or a mixture of nitrogen and a reducing gas is delivered under suitable pressure through a flexible connection 13 to the pipe 12 and is thus delivered beneath the surface of the molten metal bath 10 to effect violent agitation of the metal. This ensures the most rapid reaction of the sulphur present in 20 the molten metal with the calcium in the slag. Desulphurization proceeds in the manner described until the sulphur content of the metal has reached the desired minimum. Thereafter 25 decarburization may be effected by the addition of iron ore or by the introduction of oxygen into the body of the molten metal through the pipe 12. In the latter case, the oxygen rapidly burns out the carbon and reduces the carbon content to the desired minimum, while at the same time increasing the temperature of the molten metal.

The procedure as described is adapted to effect material savings in the production of iron and steel, especially through the more rapid transfer of the sulphur from the metal to the slag, since the reaction is not complicated by the presence of an oxidizing agent. The saving in time is important, since it increases the capacity of the equipment of a particular size, thus making the production of metal of low sulphur content more economical. The invention is particularly effective with iron containing relatively high proportions of sulphur as compared with the better grades of iron in which the sulphur content is low.

Various changes may be made in the procedure as described as well as in the apparatus employed without departing from the invention or sacrificing the advantages thereof.

We claim:

1. The method of removing sulphur and carbon from iron or steel which comprises maintaining a molten bath of the iron or steel on an open hearth furnace, maintaining a highly basic and fluid slag having a lime to silica ratio of 55 at least 2.5 to 1 on the molten bath, introducing

a non-oxidizing gaseous medium beneath the surface of the molten bath to effect agitation thereof, continuing such introduction of the non-oxidizing gas until a predetermined degree of desulphurization of the molten bath has been obtained, maintaining the molten metal free of oxidizing agents during the introduction of the non-oxidizing gaseous medium, removing the highly basic slag from the molten metal, and then decarburizing the molten bath on the same hearth in which desulphurization was obtained by introducing oxygen into the molten metal bath to combine with carbon of the molten metal and to raise the temperature of the bath.

2. A modified open hearth furnace process for removing sulphur and carbon from iron or steel which comprises maintaining a molten bath of the iron or steel in said furnace, maintaining a highly basic and fluid slag having a lime to silica ratio of at least 2.5 to 1 on the molten bath, introducing a non-oxidizing gaseous medium beneath the surface of the molten bath to effect agitation thereof, continuing such introduction of the non-oxidizing gas to change the oxidizing condition of a normal open hearth process to a neutral or slightly reducing condition until a predetermined degree of desulphurization of the molten bath has been obtained, maintaining the molten metal free of oxidizing agents during the introduction of the non-oxidizing gas, removing the highly basic slag from the molten metal, and then decarburizing the molten bath on the same hearth in which desulphurization was obtained by introducing oxygen into the molten bath to combine with the carbon of the molten metal.

FRANCIS T. CREGO.  
HAROLD R. FISHER.

40 References Cited in the file of this patent  
UNITED STATES PATENTS

| Number    | Name   | Date          |
|-----------|--------|---------------|
| 1,034,786 | Greene | Aug. 6, 1912  |
| 2,110,066 | Heuer  | Mar. 1, 1938  |
| 2,290,961 | Heuer  | July 28, 1942 |

45 OTHER REFERENCES

Report of Investigations No. 2502, U. S. Bureau of Mines, pages 31, 32, and 33.

50 Basic Open Hearth Steel Making, pages 144 and 512. Published in 1944 by the A. I. M. E., New York.

Metal Progress, December 1947, pages 963 to 967.